

# UNITED STATES PATENT OFFICE.

EDWARD D. KENDALL, OF NEW YORK, N. Y.

## ELECTROLYTICALLY TREATING SCRAP-TIN.

SPECIFICATION forming part of Letters Patent No. 656,982, dated August 28, 1900.

Application filed November 20, 1899. Serial No. 737,676. (No specimens.)

To all whom it may concern:

Be it known that I, EDWARD D. KENDALL, of the city and State of New York, have invented certain Improvements in Processes of 5 Electrolytically Treating Scrap-Tin for the Separate Recovery of Pure Iron and Tin Therefrom, of which the following is a specification.

In the processes for recovering the tin from 10 so-called "scrap tin-plate" heretofore commonly employed the iron residuum is of comparatively small value, because it is not wholly freed from tin.

The principal objects of the electrolytic 15 process herein described are to effect the complete dissociation and separate recovery of the iron and tin present in scrap tin-plate and, incidentally, to secure in commercial quantities as a by-product a nitrate of the alkali 20 metal or alkaline-earth metal the nitrate of which forms the base of the electrolyte employed. Commercial nitrate of sodium, commonly called "Chili saltpeter" is preferably employed because of its comparatively small 25 cost; but there may be employed nitrate of potassium or ammonium or calcium or any other suitable nitrate, it being understood that a nitrate which in aqueous solution, under the influence of the electric current, 30 would deposit on the cathode any metal other than tin would not be a suitable nitrate for the present purpose.

In carrying the invention into practice there is prepared an electrolyte consisting of 35 an aqueous solution containing five per cent., more or less, by weight, of the nitrate selected. The solution is usually filtered and is then introduced into an electrolytic vat, which may have any desired form or size and may be 40 made of iron or steel or of wood. The inner surface of the vat, which is exposed to contact with the solution, may, if desired, be lined with metal or coated with asphalt or suitable paint or other chemical-resisting material. 45 In appropriate relation to the electrolyte and in any desired position or positions there may be arranged a plate or plates of carbon or of tin or other metal coated with tin to serve as the cathode. It will be understood that if 50 the vat be made of metal or lined with metal such metal may in some instances be advan-

tageously made to serve as the cathode, particularly if the surfaces in contact with the electrolyte be coated with tin. The scrap tin-plate to be operated upon, which may or may not have been passed through corrugating-rolls, is loosely packed to form a mass, which is submerged in the electrolyte and made to serve as the anode by connection in the usual manner with one terminal of a charged electric circuit, the cathode being electrically connected with the other terminal of said circuit. Of course a plurality of so-prepared electrolytic vats, preferably arranged in series, may be operated together. The ensuing chemical 60 action is as follows:  $Sn + NaNO_3 + H_2O \rightarrow SnO_2 + NaNO_2 + H_2$ . The results are the formation of stannic oxid in the form of a solid precipitate, a portion of which on coming in contact with the cathode will be reduced to metallic 65 tin. A further result is the reduction to a nitrite of the sodium nitrate or other nitrate originally contained in the electrolyte. After using the electrolyte until it ceases to act with the desired energy I add enough of the 70 nitrate (say sodium nitrate) to restore efficiency to the solution. By such repeated addition the solution finally becomes heavily charged with sodium nitrite and usually contains a small proportionate quantity of 75 unchanged nitrate and also some ammonia resulting from the electrolytic decomposition of the nitrite. It may also contain traces of 80 tin, which may be recovered by electrolysis when deemed expedient. This strong solution of sodium nitrite is conducted to any 85 suitable evaporating plant in which the water present is driven off, leaving as a residuum the salts from the solution in a solid form available for use as a source of nitrogen 90 in the preparation of agricultural fertilizers.

Should the electrolytic operation have been carried so far as to have generated in the solution a material quantity of ammonia, this may be neutralized with an equivalent 95 quantity of sulfuric acid, in which case the saline mass recovered from the solution will contain some ammonia sulfate, also useful for fertilizing purposes.

The stannic oxid, which forms a precipitate in the electrolyte, and any metallic tin which may have been produced may be from

time to time collected and utilized in any of the usual ways for the production of sodium stannate or metallic tin.

It will be understood that the treatment is 5 more or less prolonged according to the greater or less size of the mass of scrap-tin submerged in the electrolyte, until the tin and iron present are completely dissociated. The sodium nitrate employed as here-  
10 in set forth is so effective an electrolytic agent that the component metals of scrap tin-plate can be completely separated within thirty minutes by the use of a six-volt electric current of adequate amperage.

15 The advantages of the described electrolytic treatment of scrap tin-plate are three-fold—to wit: first, the complete separation of the tin and the production of a pure iron having the same commercial value as like  
20 grades of iron uncontaminated with tin; secondly, the absence of any evolution from the electrolyte of any noxious or deleterious gases, and, finally, the opportunity afforded for the recovery of a valuable by-product—  
25 to wit, the described nitrite available in the manufacture of agricultural fertilizers.

What is claimed as the invention is—

1. The improvement in the art of electrolytically dissociating the iron and tin of so-  
30 called "scrap tin-plate," which consists in the preparation of an electrolyte composed of an aqueous solution of a nitrate of an alkali metal, or a nitrate of an alkaline-earth metal; the introduction into said electrolyte of an  
35 anode consisting of a mass of scrap tin-plate; the electrical connection of said mass with one terminal of a charged electric circuit and the establishment in contact with said elec-  
40 trolyte, of a suitable cathode electrically connected with the other terminal of said charged electric circuit.

2. The improvement in the electrolytic treatment of scrap tin-plate, which consists in the preparation of an electrolyte composed  
45 of an aqueous solution of a nitrate of an alkali metal, or a nitrate of an alkaline-earth metal; the introduction into said electrolyte of an anode consisting of a mass of scrap tin-

plate; the electrical connection of said mass with one terminal of an electric circuit; the 50 arrangement in contact with said electrolyte of a suitable cathode electrically connected with the other terminal of said electric circuit, and the establishment and maintenance in said circuit of an electric current until the 55 iron constituent of the anode is completely freed from the tin constituent thereof, preparatory to the separate recovery of the thus-purified iron and tin.

3. The improvement in the art of electro- 60 lytically treating so-called "scrap tin-plate," which consists in submerging an anode composed of said scrap tin-plate in an electrolyte composed of an aqueous solution of a nitrate of an alkali metal or a nitrate of an alkaline- 65 earth metal; the electrical connection of said anode with one terminal of a charged electric circuit; the establishment of a suitable cathode electrically connected with the other terminal of said charged electric circuit whereby the nitrate originally present is transformed into a nitrite; the addition of sodium or other nitrate to the solution from time to time as required, and finally, the collection and evaporation of the resulting strong solu- 70 tion for the recovery of the salt therefrom in a solid form.

4. In the electrolytic treatment of scrap tin-plate, consisting in the submergence of an anode composed of scrap tin-plate in an elec- 80 trolyte composed of an aqueous solution of sodium or other suitable nitrate, and in contact with a suitable cathode, the said anode and cathode electrically connected respectively with the opposite terminals of a charged 85 electric circuit; the introduction into the said electrolyte from time to time, as required, of additional quantities of said sodium or other nitrate, and the concentration by evaporation of the resulting strong solution for the recov- 90 ery of the nitrite therefrom.

EDWARD D. KENDALL.

Witnesses:

A. M. JONES,  
E. GATTERER.